



US006660978B1

(12) **United States Patent**  
Avdeev et al.

(10) **Patent No.:** US 6,660,978 B1  
(45) **Date of Patent:** Dec. 9, 2003

(54) **ELECTRICALLY CONDUCTING TEXTILE AND THE METHOD FOR REALIZING THE SAME**

(75) Inventors: **Oleg Valerievich Avdeev,**  
Saint-Petersburg (RU); **Tatiana Nikolayevna Genusova,**  
Saint-Petersburg (RU); **Vladimir Igorevitch Rumenstev,**  
Saint-Petersburg (RU)

(73) Assignee: **3C-Carbon and Ceramic Company B.V., Vucht (NL)**

(\*) Notice: Subject to any disclaimer, the term of this patent is extended or adjusted under 35 U.S.C. 154(b) by 0 days.

(21) Appl. No.: **09/980,984**

(22) PCT Filed: **May 1, 2000**

(86) PCT No.: **PCT/NL00/00282**

§ 371 (c)(1),  
(2), (4) Date: **Mar. 13, 2002**

(87) PCT Pub. No.: **WO00/67528**

PCT Pub. Date: **Nov. 9, 2000**

(30) **Foreign Application Priority Data**

Apr. 29, 1999 (RU) ..... 99109276

(51) **Int. Cl. 7** ..... **H05B 3/14**

(52) **U.S. Cl.** ..... **219/549, 219/548, 219/553;**  
**338/210; 427/228; 427/122**

(58) **Field of Search** ..... **219/549, 548,**  
**219/553, 545; 338/210; 252/502, 510, 511,**  
**518.1; 524/62, 79, 494; 427/249.1, 249.3,**  
**255.11, 255.14, 255.6, 314, 316, 122, 228;**  
**264/29.1, 29.4**

(56) **References Cited**

U.S. PATENT DOCUMENTS

3,949,106 A 4/1976 Araki et al.

|             |           |                              |
|-------------|-----------|------------------------------|
| 4,510,077 A | 4/1985    | Elton                        |
| 4,752,504 A | * 6/1988  | Rickborn ..... 427/249       |
| 4,825,049 A | 4/1989    | Rickborn                     |
| 4,895,082 A | 1/1990    | Mindermann et al.            |
| 5,256,177 A | * 10/1993 | Bennett ..... 65/3.11        |
| 5,373,046 A | * 12/1994 | Okamura et al. ..... 524/413 |
| 5,891,518 A | * 4/1999  | Acevedo et al. ..... 427/228 |

FOREIGN PATENT DOCUMENTS

|    |          |        |
|----|----------|--------|
| JP | 10068514 | 3/1998 |
| JP | 11094227 | 4/1999 |

\* cited by examiner

*Primary Examiner*—Teresa Walberg

*Assistant Examiner*—Shawntina T. Fuqua

(74) *Attorney, Agent, or Firm*—Handal & Morofsky

(57) **ABSTRACT**

The invention pertains to the electrothermal field and in particular to the resistive heating elements on the basis of the glass-fibre textile with the pyrocarbon coating and may be used for the production of the heating elements in heaters for both industrial and domestic applications. For obtaining the electrically conducting textile with the wide range of resistance and for broadening its sphere of application, as well as lowering the deposition temperature and retaining low scattering of the resistance along the whole field of the textile, the said textile contains 0.2–15% weight of pyrocarbon of turbostrate structure with hydrogen content up to 2% weight and with density of 0.8–1.5 g/cm<sup>3</sup>, and 86.0–99.8% weight of glass-fibre textile with the softening temperature at least 650° C. The raw hydrocarbon materials used for pyrocarbon production are hydrocarbon oils with the viscosity of 8 to 23 sSt, which are preliminarily heated to 350–450° C. and in the flow of the inert gas are put through the nozzle with the developed surface at the temperature of 450–500° C., while the deposition of the pyrocarbon out of the chemical vapour is effected at 600–800° C. with the subsequent degassing of the obtained textile at 350–450° C. in the vacuum.

**10 Claims, 3 Drawing Sheets**



Fig 1



*Fig 2**Fig 3*

*Fig 4**Fig 5**Fig 6*

**ELECTRICALLY CONDUCTING TEXTILE  
AND THE METHOD FOR REALIZING THE  
SAME**

**TECHNICAL FIELD**

The invention relates to the electrothermal field, and in particular to resistive heating elements based on a glass-fibre textile with a pyrocarbon coating and may be used for the production of heating elements in heaters for both industrial and domestic applications.

Russian Patent No. 2018492, 1992 discloses the electrically conducting materials on the basis of woven siliceous or quartz monofilaments with pyrocarbon coatings. Said coating has a width of 2 to 200 nm, and Russian Patent No. 2100914, 1996 discloses the same with a coating of pyrocarbon on the laminated structure.

However in order to obtain the known electrically conducting materials only the highly siliceous or quartz filaments with high softening temperatures could be used. This limits significantly the areas of application for the known materials as heating elements due to their high cost.

U.S. Pat. No. 4,825,049, 1989 discloses an electrically conducting textile consisting of glass-fibre with a pyrolytic carbon coating containing at least 70% of carbon, obtained via pyrolysis of hydrocarbons at temperatures of 800 to 1200° C., with the following ratio of the components, % weight:

|                          |             |
|--------------------------|-------------|
| Pyrolytic carbon coating | 0.001–17.0  |
| Glass-fibre textile      | 83.0–99.999 |

The known electrically conducting cloth has a resistance of 0.1 to 1000 Ohm/cm<sup>2</sup>.

Among the disadvantages of the known textile the following could be named: the impossibility of increasing its resistance above 1000 Ohms, which limits its field of application. Besides, the necessity to use the glass-fibre textile with softening temperature over 800° C. because of the high pyrolysis temperature also limits its field of application in various heaters because of its high cost.

Russian Patent No. 2018492, 37/00, 1992 discloses a method of production of electrically conducting materials on the basis of siliceous and quartz filaments coated with pyrocarbon layer involving the deposition of pyrocarbon out of the chemical vapor, achieved at temperature of 800 to 1000° C. out of natural gas.

Russian Patent No. 2100914, 1996 discloses a method of production of electrically conducting elements on the basis of siliceous or quartz monofilaments covered with a layer of pyrocarbon of laminated structure, involving the supply of a hydrocarbon raw material, e.g.—deoxidized white-spirit or kerosene in a flow of inert gas, nitrogen and glass filaments into the reactor with the subsequent deposition of the pyrocarbon out of the chemical vapour to the filaments' surface at the temperature of 100–1100° C.

**SUMMARY OF THE INVENTION**

The disadvantage of the known methods is the high temperature of the pyrocarbon deposition which results in impossibility of using the glass filaments with low softening temperatures in the production of electrically conducting textiles.

The purpose of the present invention is to obtain the electrically conducting textile with the wide range of resistance as well as broadening its field of application at the heating element, as well as the lowering of the temperature of the pyrocarbon deposition in order to increase the range of the glass-fibre textiles used for its production while retaining the low resistance scatter along the whole field.

The purpose is attained via the following: the known electrically conducting textile consisting of glass-fibre textile with the pyrolytic carbon coating is modified to contain a glass-fibre textile with a softening temperature not less than 640° C. and with the pyrocarbon having a paracrystalline structure with a density of 0.9–1.5 g/cm<sup>3</sup>, containing up to 2% weight of hydrogen with the following components 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9

filament which is achieved by the proposed coating technology. The above excludes the possibility of the stratification of the pyrocarbon coating and provides the uniformity of the electrical properties along the whole field of textile because the scattering of the electrical resistance along the length and across the width is within 7–10%. The claimed ration of the components in the electrically conducting textile provides the wide range of the resistance with which it could be produced.

#### BRIEF DESCRIPTION OF THE SEVERAL VIEWS OF THE DRAWINGS

FIG. 1 is an overall view of the electrically conducting textile production plant.

FIG. 2 is a C surface plot of parameters  $x_1$  and  $x_2$  against  $t$  for a given temperature and pulling velocity;

FIG. 3 is a two-component electron micrograph of a pyrocarbon-coated glass-fibre textile and a coated filament;

FIG. 4 is an IR transmission-absorption spectrum;

FIG. 5 shows X-ray photoelectron spectra of pyrocarbon coated textile and pyrographite; and

FIG. 6 shows a laser desorption spectrum of pyrocarbon-coated textile.

#### DETAILED DESCRIPTION OF THE INVENTION

Referring to FIG. 1, the plant includes the drums 1, reactor oven 2, tape pulling mechanism 3, deposition zone 4, 30 gasifier 5, nozzle 6 and vacuum oven 7.

An electrically conducting textile is proposed, containing glass-fibre textile with a softening temperature at least 640° C. with the coating of pyrocarbon of turbostrate structure having density of 0.9–1.5 g/cm<sup>3</sup>, containing up to 2% weight of hydrogen with the following components, ratio, % weight.

|                                                                 |           |
|-----------------------------------------------------------------|-----------|
| Pyrocarbon of turbostrate structure                             | 0.2–15.0  |
| Glass-fibre textile with softening temperature at least 650° C. | 85.0–99.8 |

Electrically conducting textile may have the protective coating of India rubber or other polymers.

As glass-fibre textile with the softening temperature at least 650° C. the proposed textile may contain the glass-fibre textile of aluminum-borosilicate filament (GOST 19906-83, GOST 19170-73), of magnesium-aluminosilicate filaments of KJIII-TO (TY 6-11-238-77), KT-11-TO (TY 6-48-64-91), KT-600II (TY 6-48-64-91), KJIII-290 and other brands.

As the polymer protective coating the India rubber coating of SKTN (GOST 13 835-73), SKTN-Med (TY 38.103.572-84), of copolymer "SMIROSIL" (TY 38.103.454-79) and of Kreol compound (TY 38.303.04-10-95) could be used.

The electrically conducting textile is produced in the following way.

The roll of glass-fibre textile is place into the drum 1 and pulled through the reactor oven 2 by means of tape-puling mechanism 3 at the speed, which provides the 0.5 to 5.0 hours' residence of the glass-fibre textile in the zone 4 of deposition of the reactor over 2.

The oil is supplied into the gasifier 5 of the reactor oven 2, which is heated up to 350–450° C. The vacuum oil

BM-4 (TY-38401-583-90), industrial oils I-20A and I-20 (GOST 20799-88), motor oils M8B<sub>2</sub>, M18G<sub>2</sub> etc. (GOST 8581-78), transformer oils (GOST 982-80), straw oil GOST 1666-80 etc., as well as wasted oils could be used as hydrocarbon oil.

The oil vapours generated in gasifier 5 of the reactor oven 2 along with the carrier gas nitrogen pass through the nozzle 6 of the gasifier are heated to 450–500° C. and are supplied to the deposition zone 4 of the reactor oven 2. The macroporous silica KSMG (GOST 39-56-76), stainless steel shavings and non-organic silicon carbide filaments (TY 6-02-1183-79) are used as nozzle. In the zone 4 of the reactor oven 2 the deposition of the pyrocarbon with the above stated parameters is carried out at 600–800° C.

At the outlet of the reactor oven 2 the coated glass-fibre textile is rolled on the drum 1 of the tape pulling mechanism 3, and then the obtained textile roll is loaded into the vacuum oven 7 and undergoes degassing at 350–450° C. during 1 hour. After cooling the obtained electrically conducting textile is covered with the protective polymer layer of up to 0.3  $\mu$ m.

Below are the examples of producing the proposed electrically conducting textile.

#### EXAMPLE 1

On the drum 1 of the tape-pulling mechanism 3 a roll of aluminoborosilicate glass-fibre textile with the softening temperature of 650° C. is placed. The reactor oven 2 and the gasifier 5 are blown out with nitrogen and heated to 600° C. and 350° C. respectively. Then the transformer oil GOST 982-80 having a viscosity of 8 cSt is supplied into the gasifier, the vapors if the said oil passing though the nozzle 6 of silica heated to 450° C. are fed into the zone 4 of deposition of the reactor oven 2. In the zone 4 of the deposition occurs the pyrolysis of the oil vapors with the generation of the pyrocarbon of the turbostrate structure, which is deposited on the glass-fibre textile, pulled though the said zone 4 with the speed of 5 m/hour by means of the tape-pulling mechanism 3. The obtained glass-fibre textile with the pyrocarbon coating is rolled on the drum 1, the roll of the said textile is loaded then into the vacuum oven 7 and is degassed during 1 hour at 350° C. and then is cooled. The obtained electrically conducting textile has the following composition:

|                                                                                                               |                          |
|---------------------------------------------------------------------------------------------------------------|--------------------------|
| Pyrocarbon of turbostrate structure with hydrogen content 0.2% of 2.0% and with density 0.9 g/cm <sup>3</sup> | 99.8%                    |
| Glass-fibre textile                                                                                           | 3000 Ohm/cm <sup>2</sup> |
| Resistance                                                                                                    |                          |

The scattering of the resistance along the length and across the width of the textile equals 7±0.5%. The characteristics of the obtained electrically conducting textile described in this example as well as in all the subsequent examples are given in the Table 1. Table 2 show the characteristics of the materials used and the technological parameters of the textile production method.

#### EXAMPLES 2–5

Electrically conducting textile is obtained by the same method as set forth in Example 1 but with different technological parameters of production method and the initial glass-fibre textile is substituted with aluminoborosilicate textile T-11 (example 2), magnesiumaluminosilicate glass-

fibre textile T-46 (BMII)—76 (example 3), siliceous textile KT-600II (example 4) and KJIII-290 (example 5), as well as oils used are substituted with vacuum oil BM-4 (example 2), with industrial oil H-20A (example 3), with motor oil M8B<sub>2</sub> (examples 4, 5). The resistance scattering of the textile in all examples remains within 7±0.5%.

### EXAMPLES 6, 7

Electrically conducting textile is obtained as set forth in example 1, but the obtained textile is additionally covered with the protective layer of the low-molecular India rubber CKTH 0.2 mcm wide (ex maple 6) and "KREOL" compound 0.3 mcm wide 9 example 7). The resistance scattering of the textile in all examples remains within 7±0.5% in example 6 and within 8±0.5% in example 7.

### EXAMPLES 8, 9

Electrically conducting textile is obtained as set forth in example 4, but as the nozzle the stainless steel shavings are used (example 8) or non-organic filaments of the silicon carbide whiskers (example 9). The resistance scattering of the textile in all examples remains within 9±0.5%.

In summary, development of the chemical fiber production technology accounts for the successful development of many technical fields and broad use of the new materials for domestic applications. This pertains as well to the wide range of conductive chemical fibers of the most diverse composition and usage possibilities.

Among these one should point out the carbon fibers, whose role in the development of the most advanced technical applications is not to be underestimated. Still, despite the diversity of properties and increasing scale of commercial production the price for this class of materials is rather high and prohibits their use in many domestic and technical fields of application.

The present invention presents the results of the development of the technology for production of the conductive textile by means of applying the pyrocarbon coating of pre-determined thickness upon each filament of the inexpensive commercially produced glass-fibre textiles.

The methods for deposition of the pyrolytic carbon out of the chemical vapor containing various hydrocarbons at atmospheric or lowered pressure upon different kinds of bases were actively studied since 1960-ies and continue to be studied until present.

The common disadvantage which hinders greatly the use of the materials obtained by chemical vapor deposition (CVD) is a way too high production cost which is due to the high energy-intensity of the process and use of expensive raw materials. This disadvantage may be mitigated by transition to the lower temperatures.

Still, the development of the production technology on the basis of such process could be a challenging task because of the complexity of the basic process and its sensitivity to the fluctuations of the basic parameters, such as deposition surface temperature, linear velocity of the gas stream, concentration of hydrocarbons, etc.

This fact accounts for the narrow range of the parameter values, exceeding which results in the considerable change in the properties of the obtained materials.

It is known that the velocity of formation of the single element of the thin pyrocarbon coating structure—monolayer of the hexagonal-bound carbon atoms is higher for olefines and aromatic hydrocarbons (pluribus impar) than that for linear low-molecular ones.

It has been proved empirically that the formation of the pyrolytic carbon coating using complex multi-component structure (e.g. oils) at temperatures as high as 600–650° C. occurs with the velocity which is enough for setting-up the continuous technological process for obtaining the conductive pyrocarbon layer upon the glass-fibre textile. Moreover, provided the specific set-up of the process and preparation system of reaction gas mixture one could deposit the pyrocarbon layer of the high precision-controlled sub-micrometer thickness upon each filament.

The plant for obtaining the pyrocarbon coating upon glass-fibre textiles comprises three-zone reactor oven, gasifier, dosage pump for liquid hydrocarbons' supply, tape-pulling mechanism with two drums for initial glass-fibre textile and for the final coated textile, temperature control system, and continuous textile surface resistance monitoring unit.

The chief difference of the suggested method for applying pyrocarbon coating lies in using the complex, multi-component systems, e.g. oils as the hydrocarbon raw material. Oil vapors are a mixture of unsaturated nafrene and aromatic hydrocarbons with the domination of the latter ones.

To stabilize the chemical vapor composition, meant for subsequent pyrolytic carbon deposition, oil vapors are preliminary directed through the heated catalyst nozzle with the developed surface, upon which the high-molecular hydrocarbons are decomposed, yielding the simpler components. Pyrocarbon is generated within the reactor, through which the glass-fibre textile is pulled by tape-pulling mechanism.

Thin pyrolytic carbon film is deposited upon each filament of the textile. The pyrocarbon layer thickness and composition determine the electrical resistance of the obtained textile. The specific electrical resistance measured by potentiometric method as resistance of the square fragment of the textile R (Ohm) is considered to be the chief parameter of the pyrocarbon. Generally it depends on the thickness of the coating, kind and density of the textile weave.

Pyrocarbon layer thickness is adjusted by adjusting the main technological parameters: deposition zone temperature, tape pulling velocity, gasifier temperature, oil supply rate surface area of the catalyst gasifier nozzle.

Multi-factor experiment planning methods allow taking into account the combined impact of various factors on the response function. The chief factors influencing the textile properties are: oil consumption ( $G_0$ ), deposition temperature ( $T_{dep}$ ) and gasifier temperature  $T_g$ . To these factors should be added the tape pulling speed and working surface area of the catalyst nozzle S. The last factor could only be adjusted before and not during the experiment, whereas the tape pulling speed at the present plant could only be adjusted in discreet steps from 2 to 14 m/hour. These factors are assumed to remain constant.

The specific conductivity of the textile C—the value, reverse for the resistance-to-weight gain ratio (per area textile) was selected as the response function.

The influence of the listed features non-linear character, so the second-order plane—orthogonal central compositional plane (OCCP), allowing for the separate estimation of the regression coefficients of all linear and square members as well as pair impacts was selected.

For the three-factor experiment (N=3) the  $x_1, x_2, x_3$  factor fluctuation ranges were selected:

( $x_1$ ) oil consumption  $G_0$ : 5–55 ml/hour.

( $x_2$ ) deposition temperature  $T_{dep}$ : 600–800° C.

( $x_3$ ) preparation temperature  $T_g$ : 450–550° C.

For such experiments the specific conductivity logarithm—in C was selected as a response function.

FIG. 2 in C surface for the preparation temperature  $T_g=540^\circ\text{ C}$ . and pulling velocity  $V_p=6\text{ m/hour}$ .

As it follows from the obtained results, there is a maximum oil consumption, above which the electrical conductivity of the coating drops. This is due to the existence of the threshold concentration of the hydrocarbons within the reaction zone, which, being exceeded, results in the domination of the soot-producing volumetric pyrolysis process over the surface process. As the temperature rises this threshold declines which is due to the significant heating of the reaction has and speeding-up of the pyrolysis process. As the temperature rises in the  $600\text{--}700^\circ\text{ C}$ . range the electrical conductivity of the coating increases drastically (by three orders of magnitude) which is caused by the two factors: increase of the deposited amount of carbon and change in the chemical composition and structure of the coating. It is known that during the decomposition of hydrocarbons at  $500\text{--}640^\circ\text{ C}$ . the remnants contain carbon and gumlike products comprising the condensed aromatic and naphthenic hydrocarbons, partially non-hydrogenated. Further increase of temperature from  $700$  to  $800^\circ\text{ C}$ . causes the slower decline of the electrical resistance (although the growth tempo of the deposited amount of carbon remains constant), which attests to the smaller contribution of the qualitative changes in the coating within the given temperature range. There is a minimum weight of the deposited carbon, which is required for the resistance to start declining, the said amount corresponding to the formation of the continuous film. The experimental figures for the deposited amount of the carbon and electrical resistance obtained for the textile of the similar weave, pluribus impar, are rather close one to another which is explained by the close figures for the specific surface of these textiles ( $2\text{--}3\text{ cm}^2/\text{g}$ ).

The developed mathematical model of the process of pyrocarbon film deposition upon the glass-fibre textile allows for obtaining the conductive pyrocarbon-coated glass-fibre textile with any pre-determined specific resistance within 5 to 2000 Ohm per square range.

The main features of the structural state of the low-temperature pyrocarbon films deposited by the above method upon the glass-fibre textile filaments at temperatures of  $600\text{--}800^\circ\text{ C}$ . are:

Turbostrate (paracrystalline) structure of the pyrolytic coating;

Presence of the considerable amount of technological impurities (accompanying chemical compounds).

The x-ray structural analysis of the coating material was done using the compact check-test pieces, obtained in the same reactor under the same conditions upon the flat bases of the analogous composition. The research was carried out by means of the x-ray diffractometer <<DRON-4>> (Russia) using the large-angle diffractometry method and  $\text{CuK}_\alpha$ -radiation. The results have shown that the pyrolytic carbon deposited under the above conditions is anisotropic and features only turbostrate structure—there are only extremely fuzzy /002/ and /004/ lines for the c-direction of the x-ray pattern. The pseudo-crystallite size is extremely small,  $L_c=7\text{--}10\text{ \AA}$ . These factors attest to the absence of three-dimensional ordering whereas the two-dimensional structure of the short-range order is already observed.

The electro-microscope research has shown that the conductivity of the textile with the specific resistance of 2000 to 5 Ohm is provided by the continuous pyrocarbon films having the thickness of 0.05 to 0.5 micrometers (FIG. 3).

FIG. 3a) Glass-fibre textile, pyrocarbon-coated at  $700^\circ\text{ C}$ .

FIG. 3b) single filament with coating.

The composition of the pyrocarbon films being the component of the pyrocarbon-coated glass-fibre textile was

studied using the IR-transmission-absorption spectroscopy method, which allow registering the smallest concentrations of impurities —about  $10^{13}\text{--}10^{14}\text{ 1/cm}^3$ .

Since carbon is highly absorptive material in the IR spectrum area, the transmission spectrums of the thin (up to several micrometers) pyrocarbon films deposited on the IR-transparent bases were selected to be the chief analysis method.

The base made of undoped silicon, the said base featuring the practically stable transmission rate in the 1 micrometer—60 micrometer wave range allowed for getting the comprehensive picture of the absorption spectrum of the low-temperature pyrocarbon films (FIG. 3).

FIG. 4. The complete IR-transmission-absorption spectrum of the low-temperature pyrolytic carbon film deposited upon the silicon base.

The spectrum showed no distinct absorption bands, but there are both the absorption increase in the short-wave range ( $\lambda=2\text{ micrometer}$ ), due to the inter-zone transitions, and absorption increase in the area of wave length over 10 micrometer, due to the free current carriers and through conductivity of the film.

In the high-frequency area of the spectrum there are registered only inter-zone transitions within the carbon itself. Simultaneously, the characteristic increase of the transmission into the long-wave area is observed for the pyrocarbon films within the entire spectrum range studied.

The weak bands observed in the 6–10 micrometer are of the absorption spectrums relate to the hydrocarbon bonds, but no bands in the 3 micrometer area were registered, the latter being responsible for the covalent bonds.

Thus the research resulted in the following conclusions: The carbon concentration in the pyrocarbon films which are the basis of the pyrocarbon-coated glass-fibre textile is not less than 95%.

The C-H bonds of the low-temperature pyrocarbon films have more dipolar nature than those of hydrocarbons.

The above conclusions were confirmed by other physical and chemical research methods.

The testing of pyrocarbon-coated textile was fulfilled using X-ray photoelectron spectroscopy (ESCA—5400, PHI, USA) the mass-spectroscopy with laser desorption and ionization (TOF-1, Bruker, Germany). The obtained results are compared with spectra of standard pyrographite and fullerene.

The core Cls spectrum shows the presence of the phase of pyrographite like C-C bonds and also the presence of C-H and C-O bonds whose amount depends on the certain sample (see FIG. 5a). The energy position of main pyrographite-like component is 284.5 ev, that is similar to pyrographite (284.5 eV). The valency band spectra of pyrocarbon-coated textile show some pronounced features which energy position is similar to corresponding features in valence band of fullerene (see FIG. 5b) and the general view of valency band looks like the overlapping of valency bands of pyrographite and fullerene. Thus the XPS results make it possible to propose the presence of pyrographite and fullerene like structures and their compositions with hydrogen and oxygen.

The typical mass-spectrum of laser ablation products of the samples is shown on FIG. 6. The major peaks correspond to the carbon structures in the range of 40–360 a.e.m. and their hydrogenated compounds. The fullerene's peaks (C<sub>60</sub> and C<sub>70</sub>) with weak intensity also present on mass-spectra of pyrocarbon-coated textile. The relative intensities of peaks depend on the temperature of sample manufacturing. The higher temperature of the more fullerenes and less hydrogenated carbon ions.

Thus the obtained results permit us to propose that carbon coating contain pyrographite matrix and hydrogenated carbons compounds and also small amount of fullerene itself. No evidence of oil contamination was observed.

FIG. 5: X-Ray photoelectron spectra of pyrocarbon-coated textile sample A) Core Cls spectra of pyrocarbon-coated textile-1, and pyrographite-2, B) Valency band spectra of pyrocarbon-coated textile-1, pyrographite-2, fullerene-3.

FIG. 6 Laser desorption mass-spectrum of pyrocarbon-coated textile.

According to the classification suggested by R. M. Levit the conductive fiber obtained by the above method belongs to the heterogeneous fibers, whose conductivity is ensured by means of surface coating. At the same time the obtained

C. and maximum specific power 5 kW/m<sup>2</sup> are due to the insulation stability range.

Rigid heating elements with the operating temperature up to 300° C., which provides thermal stability during the heating of the composite insulating coating. The patterns for heating large-size tanks and devices are assembled on the basis of these heaters.

Besides the above, a group of heating devices was developed and tested, which operates at extra-low safe voltage: heating floors, clothing, car set covers, etc.

The testing of these heating elements have shown their capability for operation during at least 20,000 hours without any change of electro-physical parameters.

TABLE 1

| The characteristics of the obtained electrically conducting textile |            |                     |                               |                            |                                 |                                 |  |
|---------------------------------------------------------------------|------------|---------------------|-------------------------------|----------------------------|---------------------------------|---------------------------------|--|
| Item #                                                              | % Weight   |                     | Pyrocarbon                    |                            |                                 |                                 |  |
|                                                                     | Pyrocarbon | Glass fibre textile | Hydrocarbon content, % weight | Density, g/cm <sup>3</sup> | Pyrocarbon layer thickness, mcm | Resistance, Ohm/cm <sup>2</sup> |  |
| 1.                                                                  | 0.5        | 99.5                | 2.0                           | 0.9                        | 0.1                             | 3000                            |  |
| 2.                                                                  | 2.5        | 97.5                | 1.3                           | 1.0                        | 0.3                             | 1520                            |  |
| 3.                                                                  | 2          | 98                  | 0.6                           | 1.2                        | 0.25                            | 34                              |  |
| 4.                                                                  | 15.0       | 85                  | 0                             | 1.5                        | 0.5                             | 1                               |  |
| 5.                                                                  | 4          | 96                  | 0.5                           | 1.4                        | 0.4                             | 7                               |  |
| 6.                                                                  | 0.5        | 99.5                | 2.0                           | 0.9                        | 0.15                            | 750                             |  |
| 7.                                                                  | 0.5        | 99.5                | 2.0                           | 0.9                        | 0.15                            | 750                             |  |
| 8.                                                                  | 7.7        | 92.3                | 0                             | 1.3                        | 0.4                             | 10                              |  |
| 9.                                                                  | 7.7        | 92.3                | 0                             | 1.3                        | 0.4                             | 10                              |  |

TABLE 2

| Characteristics of the materials used and technological parameters of production method |                                                    |                    |                            |                          |                              |                                    |                                                  |                             |
|-----------------------------------------------------------------------------------------|----------------------------------------------------|--------------------|----------------------------|--------------------------|------------------------------|------------------------------------|--------------------------------------------------|-----------------------------|
| Item #                                                                                  | Softening temperature of glass fibre textile, ° C. | Oil viscosity, sSt | Gasifier temperature, ° C. | Nozzle temperature, ° C. | Deposition temperature, ° C. | Residence in deposition zone, hour | Pulling speed of the glass fibre textile, m/hour | Degassing temperature, ° C. |
| 1.                                                                                      | 650                                                | 8                  | 350                        | 450                      | 600                          | 1                                  | 5                                                | 350                         |
| 2.                                                                                      | 650                                                | 8-11               | 350                        | 450                      | 600                          | 5                                  | 1                                                | 450                         |
| 3.                                                                                      | 850                                                | 17-23              | 400                        | 500                      | 700                          | 0.5                                | 10                                               | 450                         |
| 4.                                                                                      | >1000                                              | 8-11               | 450                        | 550                      | 800                          | 4                                  | 1.25                                             | 350                         |
| 5.                                                                                      | >1000                                              | 8-11               | 450                        | 550                      | 750                          | 1                                  | 5                                                | 400                         |
| 6.                                                                                      | 650                                                | 5                  | 350                        | 450                      | 600                          | 1                                  | 5                                                | 350                         |
| 7.                                                                                      | 650                                                | 8                  | 350                        | 450                      | 600                          | 1                                  | 5                                                | 350                         |
| 8.                                                                                      | >1000                                              | 8-11               | 450                        | 550                      | 700                          | 1                                  | 5                                                | 350                         |
| 9.                                                                                      | >1000                                              | 8-11               | 450                        | 550                      | 700                          | 1                                  | 5                                                | 350                         |

conductive textile meets all the strict requirements set for this class of the materials:

Low density

High physical and mechanical properties

Possibility for varying the electro-physical parameters within a broad range.

The above qualities allow for using this material for various applications including a wide scope of electrical heating elements.

As an example of the possible application, several kinds of heating elements based on this textile were developed and lab- and field-tested.

Thin flexible heating elements with the combined electrical insulation coating made of silicon sealant and polyamide film. Such heaters are designed for heating containers, pipelines with viscous liquids, chemical and medical devices, construction patterns, etc. Temperature limit 220°

What is claimed is:

1. Electrically conducting textile consisting of (a) a glass-fibre textile having a softening temperature of at least 650° C., the glass fibre textile being coated with (b) a pyrocarbon, said pyrocarbon having a paracrystalline structure, a hydrogen content up to 2% by weight and a density of 0.9 to 1.5 g/cm<sup>3</sup>, wherein (a) and (b) are present within a ratio of 85.0 to 99.8 percent by weight and 0.2 to 15.0 percent by weight, respectively.

2. Electrically conductive textile according to claim 1, wherein the electrically conductive textile has an additional protective polymer coating.

3. Method for producing an electrically conducting textile consisting of a glass-fibre textile with a pyrolytic carbon coating according to claim 1, wherein:

(a) a mixture of a raw hydrocarbon material and an inert gas is preheated to 350° C. to 450° C., said raw hydrocarbon material being a hydrocarbon oil having a

**11**

viscosity of 5 to 23 cSt, and being formed into a vapour and gas mixture,

(b) said vapour and gas mixture is supplied to a reactor through a nozzle having a temperature of 450° to 550° and is formed into a reaction gas mixture,

(c) a pyrocarbon is formed from the reaction gas mixture at a temperature of 600° to 800° C. and is deposited on the glass-fibre thereby forming a pyrocarbon coated glass-fibre textile, and

(d) the pyrocarbon coated glass-fibre textile is degassed in vacuum at a temperature of 350° to 450° C.

4. Method according to claim 3, wherein the raw hydro-carbon material is selected from the group consisting of industrial oils, motor oils, transformer oils, vacuum oils, straw oils or the wastes thereof.

5. Method according to claim 3, wherein the nozzle comprises macroporous silica, stainless steel shavings or non-organic filaments.

**12**

6. Method according to claim 3, wherein the pyrocarbon coated glass-fibre textile is coated with a protective polymer layer.

7. Method according to claim 4, wherein the nozzle comprises macroporous silica, stainless steel shavings or non-organic filaments.

8. Method according to claim 4, wherein the pyrocarbon coated glass-fibre textile is coated with a protective polymer layer.

9. Method according to claim 5, wherein the pyrocarbon coated glass-fibre textile is coated with a protective polymer layer.

10. Method according to claim 7, wherein the pyrocarbon coated glass-fibre textile is coated with a protective polymer layer.

\* \* \* \* \*